

## UNITED STATES PATENT OFFICE

2,120,740

## PRODUCTION OF IRON

Erich Faust and Eberhard Jung, Herrenwyk,  
Lübeck, Germany, assignors to Hochofenwerk  
Lübeck Aktiengesellschaft, Herrenwyk, Lübeck,  
Germany, a company of Germany

No Drawing. Application December 28, 1936, Serial No. 118,017. In Germany February 6, 1936

7 Claims. (Cl. 75—41)

This invention relates to improvements in the production of iron and is particularly concerned with the production of a crude iron containing more than 0.6% of titanium.

5 Frequent attempts have already been made to smelt iron ores containing titanium. On the one hand, it was desired to create in this fashion a profitable use for certain magnetic iron ores containing titanium, such as are found in Norway 10 for example, or Japanese titanium-iron sands for example and, on the other hand, it was intended to produce crude irons containing titanium. Although these attempts were successful in avoiding the high viscosity of the slag, which frequently 15 occurs with a normal slag-composition due to increase of the  $TiO_2$  content, by working with highly acid slag (for instance, 46%  $SiO_2+Al_2O_3$  and 44%  $CaO+MgO$ ), they did not succeed in obtaining, in continuous operation, appreciable 20 contents of titanium in the crude iron, in particular contents exceeding 0.6% (Cf. Osann, "Lehrbuch der Eisenhüttenkunde", published by W. Engelmann, 2nd edition 1923, pages 643 and 644). A crude iron with a high titanium-content was 25 first successfully produced a few years ago in the electrical blast-furnace (Bremanger A. S., Norway).

It has now been found that it is possible to produce crude iron with a higher content of titanium, 30 exceeding 0.6%, in continuous operation and without difficulty in the coke blast-furnace provided that certain conditions are observed in regard to the slag-composition and furnace-temperature. With a slag which consists, as is usual, 35 of calcium silicates, experience shows that an appreciable reduction of  $TiO_2$  does not occur; furthermore there is also the danger of extra-ordinarily difficult fusibility and consequently of trouble with the furnace. If, however, a slag is 40 employed which consists predominantly of calcium aluminates, that is predominantly of compounds of  $CaO$  and  $Al_2O_3$ , then it is possible to reduce considerable quantities of the titanic 45 oxide and to transfer it into the crude iron. A condition is that high hearth-temperatures, which amount to more than 1600° C. and frequently up to 1800° C. and more, are operated with. In this fashion, it is possible to transfer up to 60% of the 50 titanium-content of the mixture or charge into the crude iron. If the process is conducted, in the known manner, with a lower hearth-temperature, then it is not possible to introduce substantial quantities of titanium into the crude 55 iron; on the contrary, by far the predominating

part of any titanium present in the mixture goes into the slag.

In order to ensure the desired slag-composition, which should as far as possible lie within the limits of 4—25%  $SiO_2$ , 35—55%  $CaO$  and 30—60%  $Al_2O_3$ , it is preferable to work with bauxite as ore. As this raw material contains, say, 3—5% of  $TiO_2$ , an addition to the mixture of titanium ores, such for example as ilmenite or rutile, is not necessary or is only necessary to a very limited extent. In 10 this manner, a high degree of economy is ensured for the process.

Moreover, it has been found, on the one hand, that it is necessary, for the good quality of the crude iron produced, to work with large quantities of slag, which may amount to three times the quantity of crude iron and, on the other hand, that the regular operation of the furnace is not endangered by slag-difficulties in spite of this 15 large quantity of slag.

Since bauxite, as an ore, contains only a little iron, it has proved advantageous to add scrap-iron to the mixture in order to increase the yield of crude iron. The de-oxidizing action of the lime-aluminate slag and of the high titanium 20 content of the crude iron nevertheless ensures for the iron a very excellent quality which is especially suitable for very highly stressed castings.

The following examples may be given to indicate the composition of the mixture.

## EXAMPLE 1

## Mixture with ilmenite

|           | Kgs. 35 |
|-----------|---------|
| Bauxite   | 3,000   |
| Ilmenite  | 300     |
| Scrap     | 3,750   |
| Limestone | 3,000   |
|           | 40      |

## EXAMPLE 2

## Mixture without separate titanium ore

|           | Kgs.  |
|-----------|-------|
| Bauxite   | 3,000 |
| Scrap     | 1,700 |
| Limestone | 3,000 |

In both cases, a crude iron with 0.8—1.7% of titanium is obtained, depending upon the furnace-temperature.

We claim:

1. In the process for the production of a crude iron containing more than 0.6% of titanium in a coke blast furnace by employment of a charge mixture of bauxite containing titanium, limestone and coke and by employment of a slag 55

- containing more than 50% of lime-aluminates and working at a furnace temperature between 1600° C. to 1800° C., the step of working with a high slag to iron ratio, which exceeds 1:1 and 5 may even be as high as 3:1 ratio.
2. The process for the production of a crude iron containing more than 0.6% of titanium in the coke blast furnace comprising charging a mixture of bauxite and titanium ores, limestone 10 and coke, employing a slag containing more than 50% of lime-aluminates and working at a furnace temperature between 1600° C. and 1800° C. with a slag to iron ratio between 1:1 and 3:1.
3. The process of claim 1 in which scrap is 15 added to the charge mixture.

4. The process of claim 1 in which the charge mixture comprises bauxite, titanium ore, limestone and coke.

5. The process of claim 2 in which the charge mixture comprises bauxite, titanium ore, limestone, scrap and coke. 5

6. The process of claim 2 in which the charge mixture comprises an aluminum containing ore, titanium ore, limestone and coke.

7. The process of claim 2 in which the charge 10 mixture comprises an aluminum containing ore, titanium ore, limestone, scrap and coke.

ERICH FAUST.  
EBERHARD JUNG. 15